

## UNITED STATES PATENT OFFICE

2,369,028

## TREATING OF NONFERROUS MATERIALS

Louis S. Deitz, Jr., Westfield, N. J., assignor to  
Nassau Smelting & Refining Company, Incorporated,  
New York, N. Y., a corporation of New York

No Drawing. Application December 14, 1943,  
Serial No. 514,275

20 Claims. (Cl. 75—24)

This invention relates to the treating of non-ferrous materials and more particularly to the production of copper base products containing substantial quantities of tin by treating non-ferrous materials and secondary metals.

It has been customary to treat materials containing copper and one or more of the metals tin, lead and zinc to utilize the metal values therein in the production of ingots of predetermined compositions. Relatively impure materials of this nature are smelted in a blast furnace to produce blast furnace pigs that are treated subsequently in a reverberatory or other furnace to refine them further. Such blast furnace pigs generally contain only a small amount of tin, seldom as much as 5%, and when they are used in reverberatory charges to make alloys containing substantial quantities of tin, virgin tin is added to the charges to increase the tin contents of the finished alloys.

It has been the practice to make in a reverberatory furnace products such as those consisting of 85% of copper, 5% of tin, 5% of lead and 5% of zinc, or 80% of copper, 10% of tin and 10% of lead, or 88% of copper, 8% of tin and 4% of zinc, respectively. The charges fed into the reverberatory furnace usually included such materials as blast furnace pigs, copper and bronze wire, brass and bronze turnings, metallic copper, tin and zinc, slags from previous charges, and the usual slagging and reducing materials.

The composite analyses of the metal values of these materials, other than the metallic tin, are such that the products obtained therefrom would contain insufficient tin to produce high tin ingots if virgin tin were not added to the charge. However, the supply of virgin tin is limited and its use is restricted. Consequently, when non-ferrous alloys containing tin are produced, it is desirable to employ processes in which some of the required tin may be supplied from other sources. Thus, there is need for processes in which the tin content of blast furnace pigs and of reverberatory or other types of ingots can be increased without the use of metallic tin.

It is an object of this invention to provide new and useful processes for treating non-ferrous materials.

In accordance with one embodiment of the invention, a suitable furnace is charged with materials containing copper and other non-ferrous metals, together with the usual slagging and reducing materials, and the materials are heated to a temperature high enough to cause the operation to proceed. Zinc-bearing material, such as

scrap brass and briquettes of zinc spelter, is included as part of the charge and tin-oxide material, such as high tin drosses and tin ores, are also incorporated in the charge, the zinc-bearing material being present in sufficient quantity to reduce a substantial portion of the tin oxide to metallic tin.

This process is based on the observation that when metallic zinc and tin oxide are heated to a temperature above the melting point of copper, the zinc reduces the tin oxide to metallic tin and the reaction proceeds exothermically. This indicated that zinc could be used as an active reducing agent for tin oxide in metallurgical processes, such as in blast furnace smelting operations and reverberatory refining processes, because the heat of reaction tends to accelerate the reaction. From this observation it was conjectured that, if a mixture of tin oxide and brass, or other 10 alloy or mixture of copper and zinc (with or without the presence of other materials, such as lead), is heated to a temperature above the melting point of copper, the zinc should reduce the tin oxide to metallic tin, and that the tin would 15 alloy with the copper. Under normal operations of this nature in accordance with this invention, where tin oxide is present in the charge, a reducing agent, such as coke, is always added to the charge and this reducing agent will reduce 20 a considerable portion of the tin and other metal oxides in the charge. In accordance with this invention, the zinc present should be sufficient to insure substantially complete reduction of any tin oxide not otherwise reduced. Experiments have 25 demonstrated that this process may be used with extremely satisfactory results on a commercial scale in commercial furnaces, and that it provides an economical and readily controlled means 30 of producing copper base alloys having high tin 35 contents.

Such a process has the advantage that the metallic tin produced is taken up by the copper and is not volatilized. Only a relatively small amount of tin is collected in flue dusts and the 40 slag contains very little tin. Consequently, tin-oxide materials containing high percentages of tin may be used to build up the tin content of the resulting product without excessive loss of tin, and this process permits the use of high tin 45 drosses and ores which formerly were not treated in blast furnaces and reverberatory furnaces used to make copper base materials. Thus, products having high tin contents may be made without the use of metallic tin.

The above-described and other objects and

features of the invention will be apparent from the following description of specific examples of processes embodying the invention, in which tin ore is used to supply a portion of the tin required to make tin-containing copper base alloys in a reverberatory furnace.

*Example I*

In accordance with this embodiment of the invention, the process was performed in such manner as to make ingots containing approximately 88% of copper, 6% of tin, 1.5% of lead and the balance zinc. This was accomplished by feeding into a reverberatory furnace charges containing various scrap materials, such as brass and bronze turnings, reclaimed wire, metallic zinc, tin-containing cable sheaths, and tin oxide ore, together with the usual reducing and slagging materials, such as coke, sand and soda ash, and heating the charge.

A typical run of this nature was carried out with the use of a charge containing the following materials:

| Pounds added | Material                        | Approximate composition |             |             |             |
|--------------|---------------------------------|-------------------------|-------------|-------------|-------------|
|              |                                 | Per cent Cu             | Per cent Sn | Per cent Pb | Per cent Zn |
| 34,530       | Special blast furnace pigs      | 82                      | 8           | 2.5         | Bal.        |
| 21,300       | Burned bronze wire              | 95                      | 1.5         | -----       | -----       |
| 11,593       | 90-10 brass turnings            | 90                      | -----       | -----       | 10          |
| 7,804        | Metal grindings                 | 67                      | 5           | 1.5         | 1           |
| 4,358        | Phosphor bronze solids          | 88                      | 1.5         | -----       | -----       |
| 10,900       | High grade turnings             | 85                      | 5           | 2.5         | 2           |
| 4,411        | Miscellaneous grade turnings    | 84                      | 4           | 2           | 2           |
| 4,340        | High grade composition scrap    | 86                      | 4           | 2.5         | 4           |
| 5,660        | High grade composition turnings | 85                      | 5           | 2           | 2           |
| 5,646        | Composition turnings            | 79                      | 3           | -----       | (68 Ni)     |
| 498          | Monel scrap                     | 30                      | -----       | -----       | -----       |
| 5,680        | Reverberatory furnace scrap     | 87                      | 7           | 2.5         | Bal.        |
| 2,064        | Bolivian tin concentrates       | 66                      | -----       | -----       | -----       |
| 560          | Pig tin                         | 100                     | -----       | -----       | -----       |
| 2,800        | Briquetted zinc                 | -----                   | -----       | -----       | 99          |
| 105          | 3% tin-lead cable sheath        | 3                       | 97          | -----       | -----       |

Approximately 1,200 pounds of coke, 550 pounds of sand and 1,700 pounds of soda ash were also employed as reducing and slagging ingredients. The tin ore was mixed with about 300 pounds of lime and 100 pounds of fine charcoal to produce a pasty mass which could be readily handled and to retard volatilization of the tin. If desired, the tin oxide ore may be briquetted with a bituminous or other cementitious material before it is introduced into the furnace.

The special blast furnace pigs contained about 8% or more of tin, while the Bolivian tin concentrates contained 66% of tin. The ingots produced analyzed an average of 88.9% of copper, 5.6% of tin and 1.5% of lead, with the balance being zinc.

About 20% of the tin required to make the alloy of this composition came from the tin ore included in the charge, and about 40% was derived from the special blast furnace pigs, while the rest was provided by the tin contents of the scrap metals treated and the 560 pounds of pig tin added to the charge. The reducing and slagging reagents, such as coke, charcoal, sand, lime, soda ash, and the like, employed, and the amounts thereof, were not substantially different than are used in the usual reverberatory furnace processes in which no tin ore is added.

Heretofore, it had not been considered commercially feasible to add substantial quantities of materials, such as ores, having high tin oxide contents, to reverberatory furnace charges of this

nature, because it would be anticipated that an excessive amount of the tin would go off as slag and as fume, which would be collected in the flue dusts. It also would be anticipated that the normal reverberatory furnace charges contain insufficient reducing material to reduce these high tin-oxide materials to metallic tin.

In accordance with the processes embodying this invention, the reverberatory charge is so adjusted that there is sufficient zinc therein to insure the substantially complete reduction of all of the tin oxide present in the charge, including that found in the tin ore. The nascent zinc vapors produced in the charge permeate the charge and effectively reduce the tin oxide not otherwise reduced to metallic tin, which immediately combines with the molten copper produced to form a copper-base alloy containing tin.

If it is desired to produce ingots containing more than about 6% of tin, this can be accomplished by adding to the reverberatory furnace charges larger quantities of tin ores and making certain that the zinc content of the charge is sufficiently high to insure substantially complete reduction of the tin oxide contained in the ore. It is also possible to use iron-free tin drosses containing upward of 40% of tin oxide instead of the tin ore, if desired. By the use of greater quantities of high tin oxide materials, ingots containing from 8% to 10% tin may be produced. If a lead-free alloy is to be made, the charge is made up of materials that contain little, if any, lead.

*Example II*

In accordance with this embodiment of the invention, a charge of the following composition was fed into a reverberatory furnace and treated in a manner similar to that described in Example I:

| Pounds added | Material                        | Approximate composition |             |             |             |
|--------------|---------------------------------|-------------------------|-------------|-------------|-------------|
|              |                                 | Per cent Cu             | Per cent Sn | Per cent Pb | Per cent Zn |
| 42,058       | Special blast furnace pigs      | 82                      | 8           | 2.5         | Bal.        |
| 10,560       | Scrap bronze wire               | 95                      | 1.5         | -----       | -----       |
| 9,000        | 90-10 brass turnings            | 90                      | -----       | -----       | 10          |
| 15,000       | Composition turnings            | 78                      | 5           | 1           | -----       |
| 3,294        | Tin residues                    | -----                   | 58          | -----       | -----       |
| 9,534        | #2 copper                       | 97                      | -----       | 2           | -----       |
| 8,370        | Scrap copper wire               | 99                      | -----       | -----       | -----       |
| 5,232        | #2 high grade composition scrap | 87                      | 6           | 2           | Bal.        |
| 956          | Bolivian tin concentrates       | 66                      | -----       | -----       | -----       |
| 2,740        | Briquetted zinc                 | -----                   | -----       | -----       | 99          |
| 200          | 3% tin-lead cable sheath        | 3                       | 97          | -----       | -----       |

About 500 pounds of charcoal, 800 pounds of coke, 650 pounds of sand and 1,500 pounds of soda ash were also added. The tin ore contained 66% of tin and was mixed with lime and charcoal, as in the previous example, before it was introduced into the furnace. The special blast furnace pigs contained about 8% of tin.

The ingots produced contained 88.01% of copper, 5.81% of tin, and 1.54% of lead, with the balance being zinc. Almost 50% of the tin in the ingots was supplied by the special blast furnace pigs, while about 10% of the tin came from the tin ore. The remainder of the tin in the ingots was provided by the tin contents of the scrap metals treated and by the tin residues which supplied slightly more than 25% of the tin. It will be observed that no pig tin was added to this charge and that the entire tin content of the ingots was obtained from secondary sources and from tin ore.

The special blast furnace pigs containing about 8% of tin, which were employed in making up the above-described charges, were made by a modification of this process in which tin oxide ores or high tin oxide drosses were added to a blast furnace charge containing sufficient zinc to insure the substantially complete reduction of the tin oxide contained in the ore or dross. This process is disclosed and claimed specifically in application Serial No. 514,274, filed Dec. 14, 1943, by L. S. Deitz, Jr., and W. H. Jacobson.

By utilizing these high tin oxide containing materials in blast furnace charges containing the requisite amount of zinc, blast furnace pigs containing 10% or more of tin can be obtained. With the usual blast furnace charge, in which the materials employed contain relatively small quantities of tin, the pigs produced contain from about 2% to not over 5% of tin.

Thus, this invention contemplates generally the utilization of high tin oxide materials in non-ferrous metal refining processes in which such materials had not formerly been used, coupled with the inclusion in the furnace charges of zinc-bearing material in sufficient quantities to cause substantially all of the otherwise unreduced tin oxide in the tin-containing materials to be substantially completely reduced thereby. The invention further contemplates the use of high tin oxide materials in a blast furnace to produce high tin blast furnace pigs, followed by the utilization of such pigs in reverberatory furnace charges which also contain high tin oxide materials to produce ingots having the desired tin content, without the introduction of more than a relatively small amount of pig tin to the reverberatory furnace charge.

It has been difficult to utilize certain tin ores, because of the relatively high percentages and the type of impurities, such as iron, found therein. In smelting such ores to produce pig tin, it has been necessary to mix them with the purer Malayan type ores. The processes embodying this invention provide means for utilizing these impure ores with a substantially complete recovery of the tin values therein, and without having to mix them with other higher grade ores.

Obviously, this invention is not limited to the use of the specific ores recited in the examples given hereinabove, but the processes embodying the invention may be practiced with satisfactory results by using other tin-bearing materials containing substantial percentages of tin oxide. By carrying out the processes in such manner that the furnace charges always contain enough zinc to insure the reduction of the tin oxide in the tin-bearing materials employed, a commercially complete reduction of the tin oxide is obtained and the losses of tin in the slag and the amount of tin appearing as a constituent of the flue dust are sufficiently low to make the process commercially feasible.

What is claimed is:

1. The process of treating non-ferrous materials which comprises introducing into a furnace a charge including fluxing and reducing materials and material containing copper, zinc and tin, and heating the charge to recover the metallic values therein, at least a substantial part of the tin-containing material being one having a high tin oxide content and the amount of zinc-containing material present being sufficient to insure the reduction to metallic tin of a substantial quantity of tin oxide.

2. The process of treating non-ferrous mate-

rials which comprises introducing into a furnace a charge including fluxing material, carbonaceous reducing material and material containing copper, zinc and tin, and heating the charge to recover the metallic values therein, at least a substantial part of the tin-containing material being one having a high tin oxide content and the amount of zinc-containing material present being sufficient to insure the reduction to metallic tin of a substantial quantity of tin-containing material which otherwise would remain unreduced.

3. The process of treating non-ferrous materials which comprises introducing into a furnace a charge including fluxing and reducing materials and material containing copper, zinc and tin, and heating the charge to recover the metallic values therein, at least a substantial part of the tin-containing material being a tin ore having a high tin oxide content and the amount of zinc-containing material present being sufficient to insure the reduction to metallic tin of a substantial quantity of tin oxide.

4. The process of treating non-ferrous materials which comprises introducing into a furnace a charge including fluxing and reducing materials and material containing copper, zinc and tin, and heating the charge to recover the metallic values therein, at least a substantial part of the tin-containing material being an iron-free tin dross having a high tin oxide content and the amount of zinc-containing material present being sufficient to insure the reduction to metallic tin of a substantial quantity of tin oxide.

5. The process of treating non-ferrous materials which comprises introducing into a furnace a charge including fluxing and reducing materials and material containing copper, zinc and tin, and heating the charge to recover the metallic values therein, at least a substantial part of the tin-containing material being one having a tin oxide content of upward of 40% and the amount of zinc-containing material present being sufficient to insure the reduction to metallic tin of a substantial quantity of tin oxide.

6. The process of treating non-ferrous materials which comprises introducing into a furnace a charge including fluxing and reducing materials and material containing copper, zinc and tin, and heating the charge to recover the metallic values therein, at least a substantial part of the tin-containing material being a tin oxide ore containing at least 60% of tin and the amount of zinc-containing material present being sufficient to insure the reduction to metallic tin of a substantial quantity of tin oxide.

7. The process of treating non-ferrous material which comprises introducing into a reverberatory furnace a charge including fluxing material, carbonaceous reducing material and material containing copper, zinc and tin, and heating the charge to recover the metallic values therein, at least a substantial part of the tin-containing material being one having a high tin oxide content and the amount of zinc-containing material present being sufficient to insure the reduction to metallic tin of a substantial quantity of tin oxide.

8. The process of treating non-ferrous materials, which comprises introducing into a furnace a charge including copper-bearing and other materials containing non-ferrous metals in such proportions as to produce an ingot metal consisting principally of copper, including in the charge a sufficient quantity of high tin oxide material to materially increase the tin content of the in-

got metal and sufficient zinc-bearing material to insure the reduction to metallic tin of a substantial quantity of tin oxide which would be unreduced, and heating the charge, whereby the nascent zinc produced assists in the reduction of the tin oxide material.

9. The process of treating non-ferrous materials which comprises feeding into a reverberatory furnace a charge including copper-bearing and other materials containing metal of the group consisting of lead, zinc and tin in such proportions as to produce an ingot metal consisting of upward of 70% of copper, including in the charge a substantial quantity of zinc-bearing material and material containing upward of 40% of tin oxide, and heating the charge, the nascent zinc derived from the zinc-bearing material assisting in the reduction of a substantial quantity of the tin oxide in the tin oxide material.

10. The process of producing tin-containing ingots without the use of substantial quantities of metallic tin, which comprises smelting in a blast furnace a charge including copper, zinc and tin-bearing materials in which a substantial part of the tin-bearing material is one having a high tin-oxide content and in which sufficient zinc-containing material is present to insure the reduction of a substantial quantity of the tin oxide in the charge to metallic tin, whereby a high tin blast furnace metal is produced, introducing such blast furnace metal into a reverberatory furnace together with material containing copper, zinc and tin, including in the reverberatory furnace charge a tin-containing material having a high tin oxide content and zinc-containing material in sufficient quantity to insure the reduction to metallic tin of a substantial amount of the tin oxide in the charge, and heating the reverberatory charge.

11. The process of producing tin-containing ingots, which comprises smelting in a blast furnace a charge including copper, zinc and tin-bearing materials, in which a substantial part of the tin-bearing material is one having a high tin oxide content and in which sufficient zinc-containing material is present to insure the reduction of a substantial quantity of the tin oxide in the charge to metallic tin, whereby a high tin blast furnace metal is produced, introducing such blast furnace metal into a reverberatory furnace together with material containing copper, zinc and tin, including in the reverberatory furnace charge a substantial quantity of tin oxide ore and zinc-containing material in sufficient quantity to insure the reduction to metallic tin of a substantial amount of the tin oxide in the charge, and heating the latter charge.

12. The process of producing tin-containing ingots, which comprises smelting in a blast furnace a charge including copper, zinc and tin-bearing materials, in which a substantial part of the tin-bearing material is one having a high tin oxide content and in which sufficient zinc-containing material is present to insure the reduction of a substantial quantity of the tin oxide to metallic tin, whereby a high tin blast furnace metal is produced, introducing such blast furnace metal into a reverberatory furnace together with material containing copper, zinc and tin, including in the reverberatory furnace charge a substantial quantity of tin oxide ore having a tin content of upward of 60% and zinc-containing material in sufficient quantity to insure the reduction of a substantial amount of the tin oxide

in the tin oxide material, and heating the latter charge.

13. The process of producing tin-containing ingots without the use of metallic tin, which comprises smelting in a blast furnace a charge including copper, zinc and tin-bearing materials, in which a substantial part of the tin-bearing material is one having a tin content of upward of 40% and in which sufficient zinc-containing material is present to insure the reduction of a substantial quantity of the tin oxide to metallic tin, whereby a high tin blast furnace metal is produced, introducing such blast furnace metal into a reverberatory furnace together with material containing copper, zinc, and tin, including in the reverberatory furnace charge a tin oxide ore having a tin content of upward of 60%, also including in the reverberatory furnace charge zinc-containing material in sufficient quantity to insure the reduction to metallic tin of a substantial amount of the tin oxide which otherwise would be unreduced, and heating the reverberatory furnace charge.

14. The process of producing tin-containing ingots with the use of a minimum amount of metallic tin, which comprises smelting in a blast furnace a charge including copper, zinc and tin-bearing materials, including in the blast furnace charge a sufficient quantity of tin-bearing material having a tin content of upward of 40% to produce a blast furnace metal having a tin content of upward of 5%, also including in the blast furnace charge sufficient zinc-containing material to reduce to metallic tin a substantial quantity of tin oxide which otherwise would be unreduced, introducing such blast furnace metal into a reverberatory furnace together with material containing copper, zinc and tin, including in the reverberatory furnace charge a tin oxide ore having a tin content of upward of 60%, also including in the reverberatory furnace charge zinc-containing material in sufficient quantity to reduce to metallic tin a substantial quantity of tin oxide which otherwise would be unreduced, and heating the reverberatory furnace charge to a temperature sufficiently high and for a period sufficiently long to recover the metallic values in the charge.

15. The process of treating non-ferrous materials, which comprises introducing into a furnace a charge including carbonaceous reducing material and material containing copper, zinc and tin, and heating the charge to recover the metallic values therein, at least a substantial part of the tin-containing material in the charge being one having a high tin oxide content and the amount of zinc-containing material present in the charge being sufficient to insure substantially complete reduction to metallic tin of the otherwise unreduced tin oxide in the charge.

16. The process of treating non-ferrous materials, which comprises introducing into a furnace a charge including carbonaceous reducing material and copper-bearing and other materials containing non-ferrous metals in such proportions as to produce a metal consisting principally of copper, including in the charge a sufficient quantity of high tin oxide material to materially increase the tin content of the metal produced and sufficient zinc-bearing material to insure the reduction to metallic tin of substantially all tin-bearing material in the charge which otherwise would be unreduced, and heating the charge.

17. The process of treating non-ferrous materials, which comprises introducing into a furnace

a charge including carbonaceous reducing material and material containing copper, zinc and tin in such proportions as to produce a copper base metal containing more than 5% of tin, and heating the charge to recover the metallic values therein, at least a substantial part of the tin-containing material in the charge having a tin oxide content of upward of 40% and the amount of zinc-containing material present in the charge being sufficient to insure the substantially complete reduction to metallic tin of the otherwise unreduced tin oxide in the charge.

18. The process of treating non-ferrous materials, which comprises feeding into a furnace a charge including carbonaceous reducing material and copper-bearing and other materials containing metals of the group consisting of lead, zinc and tin in such proportions as to produce a metal consisting of upward of 70% of copper and more than 5% of tin, including in the charge a substantial quantity of zinc-bearing material and tin oxide material containing upward of 40% of tin oxide, and heating the charge, the nascent zinc derived from the zinc-bearing material effecting the reduction of a substantial quantity of the tin oxide in the charge which otherwise would be unreduced.

19. The process of treating non-ferrous material, which comprises introducing into a reverberatory furnace a charge including carbonaceous reducing material and material containing copper, zinc and tin, and heating the charge to

recover the metallic values therein, a substantial part of the tin-containing material in the charge being a tin ore having a high tin oxide content and the amount of zinc-containing material present in the charge being sufficient to insure substantially complete reduction to metallic tin of the otherwise unreduced tin oxide in the charge.

20. The process of producing tin-containing ingots, which comprises smelting in a blast furnace a charge including carbonaceous reducing material and copper, zinc and tin-bearing materials in such proportions as to produce a blast furnace metal consisting principally of copper and containing in excess of 5% of tin, in which charge a substantial part of the tin-bearing materials has a high tin oxide content and the amount of zinc-containing material is sufficient to insure substantially complete reduction to metallic tin of the otherwise unreduced tin oxide in the charge, introducing such blast furnace metal into a reverberatory furnace as part of a charge including carbonaceous reducing material and materials containing copper, zinc and tin, in which reverberatory furnace charge a substantial part of the tin-containing material has a high tin oxide content and the amount of zinc-containing material present is sufficient to insure substantially complete reduction to metallic tin of the otherwise unreduced tin oxide in the charge, and heating the reverberatory charge.

LOUIS S. DEITZ, JR.